

## UNITED STATES PATENT OFFICE.

ARTHUR C. DAVIDSON, OF BRONXVILLE, NEW YORK, ASSIGNOR TO D. CO., INC., OF NEW YORK, N. Y., A CORPORATION OF NEW YORK.

## ALLOY STEEL.

No Drawing. Application filed October 28, 1919. Serial No. 333,987.

To all whom it may concern:

Be it known that I, ARTHUR C. DAVIDSON, a citizen of the United States, and a resident of Bronxville, in the county of Westchester and State of New York, have invented certain new and useful Improvements in Alloy Steel, of which the following is a specification.

This invention relates to alloy steel and has for its object to provide a steel which can be cast directly from the melt into tools such as for turning, milling cutters, countersinks, reamers, dies, bar stock, etc., of only slightly greater section than the finished article, and only requiring to be finished by grinding and heat treatment, without the forging, rolling and machining operations now customarily employed in finishing into tools steel from ingots. Besides a saving in labor of up to 90%, this invention provides a steel which outlasts the best brands of forged steel now on the market by from two to upwards of ten times, requires less frequent grinding, and will work at higher cutting speeds than are at present considered practicable.

Such a steel must be homogeneous, of character to properly fill in the mold, and capable of being cast with a minimum loss in usable castings from heads and risers.

A crucible steel cast at 3400° F. and upwards and varying in analysis between the percentage limits given below, according to the duty to be performed, has given extremely successful results in practice: tungsten, 14.00-22.00; vanadium, .50-3.00; chromium, 2.00-12.00; zirconium, .50-6.00; cobalt, 1.00-8.00; carbon, .35-1.25, the balance being iron, and impurities, in which latter class I include silicon and manganese, which may vary from .02 to 1.30, and .05 to 1.00, respectively, without material effect on the results. Minute traces of phosphorus and sulphur may also be found in the analysis, depending on the purity of materials used for the base, the material of the crucible, etc. Vanadium or cobalt, or both, may be omitted in some instances without detriment to the steel for special purposes, but cutting tools are improved by including both.

An analysis suitable for lathe tools, tool

holder bits, etc., in percentages, is tungsten, 18.00; vanadium, 1.50; chromium, 7.00; zirconium, 1.00; cobalt, 5.00; carbon, .65.

The iron should generally be 60%. With the higher percentages of tungsten, etc., this steel will readily forge with ordinary methods and special care, but at the lower range of heat it is only forgeable with difficulty and care, but this does not improve the cutting qualities materially. Forging ordinarily will injure them, owing to setting up of strains, cracks, etc., which annealing will not remove, but which will develop after quenching, or in use.

The steel is cast at from 3200° F. upward, and sharply fills out the mold without excess shrinkage, and consequently does not necessitate a large head, which is useless in the tool and involves waste of metal. In many cases risers are not even required, owing to the extreme fluidity of this alloy, which continues for an unusual time in the mold, as compared with ordinary steels. When taken out of the mold, the castings may be cleaned and annealed, then ground, heated to 2200° F. or upward, then quenched, preferably in oil, and drawn at about 800° F., or as the experience of the hardener after a few tests will indicate. No checks or cracks develop during this treatment, which often occur with forged steel and castings even when treated at a lower temperature. The tool is then ground to size ready for use. Sand molds may be used, rammed hard either in a machine or by hand, and give very sharp and accurate castings.

I claim:

1. Alloy steel comprising zirconium in combination with iron, tungsten, chromium and vanadium between the limits of the proportions specified.

2. Alloy steel comprising zirconium in combination with iron, tungsten, chromium, cobalt and vanadium between the limits of the proportions specified.

3. A cast alloy steel cutting tool ready for use after grinding and heat treatment without rolling, forging or machine cutting work comprising iron, tungsten, chromium, cobalt and zirconium between the limits of the proportions specified.

4. A cast alloy steel cutting tool ready for use after grinding and heat treatment without rolling, forging or machine cutting work comprising iron, tungsten, chromium, cobalt, vanadium and zirconium between the limits of the proportions specified.
5. Alloy steel comprising tungsten 18%, vanadium 1.5%, chromium 7%, zirconium 1%, cobalt 5%, and carbon .65%, in combination with iron.

Signed at the city of New York, in the county and State of New York, this 24th day of October, A. D. 1919;

ARTHUR C. DAVIDSON.